# EUROPEAN PATENT SPECIFICATION

(11) **EP 0 509 971 B1**
(45) Date of publication and mention of the grant of the patent: **27.09.1995**
(21) Application number: 92830186.0
(22) Date of filing: 16.04.1992
(51) Int. Cl.: C22C 24/00, H01J 7/18

(54) **A process for the sorption of residual gas and especially nitrogen gas by means of a non-evaporated barium getter**
Verfahren zur Sorption von Restgasen, insbesondere von Stickstoff mittels eines nichtverdampfbaren Bariumgetters
Procédé pour l'absorption de gaz résiduels, en particulier pour l'azote, avec mise en oeuvre d'un getter non-évaporé au baryum

(30) Priority: 16.04.1991 IT MI911038
(43) Date of publication of application: 21.10.1992
(73) Proprietor: SAES GETTERS S.p.A., I-20123 Milano (IT)
(72) Inventor: Boffito, Claudio, I-Rho (Milano)) (IT); Schiabel, Antonio, I-Garbagnate (Milano) (IT)
(74) Representative: Adorno, Silvano

(56) References cited:
- EP-A- 0 226 244
- GB-A- 387 724
- GB-A- 2 161 322
- US-A- 2 706 554
- US-A- 3 193 508

## Description

The present invention relates to a process for a sorbing residual gases by means of a non-evaporated barium getter.

Barium getters are well known in the art. In the form of the more of less pure element, barium was placed inside a metal container to protect it from reaction with the atmosphere. Then, when required to be used, it was mounted inside a vacuum device where, after partial evacuation and seal-off of the device, the barium was caused to evaporate. The barium, after evaporation, deposited in the form of a thin film within the vacuum device where it sorbed the residual or unwanted gases throughout the life of the device.

While these getter devices released barium they were also found to release a large amount of undesirable gases that had been picked up during storage or handling. This was due to the getter material being barium in the form of an element which is reactive with gases.

In order to reduce the reactivity of the barium, it was then alloyed with one or more metals. Such alloys were *inter alia* Ba-Mg, Ba-Sr-Mg, Ba-Mg-Al. See for example the book "Getterstoff und Ihre Anwendung in the Hochvakuumtechnik" by M. Littmann, E Winter'sche Verlagshandlung, Leipzig 1939. One of the most successful was the alloy BaAl₄ having a weight percent of barium from 40 to 60 percent. Such an alloy is very inert and, as with all inert barium alloys, it must be evaporated before it can sorb gases. It can be caused to dissociate and release barium by means of applying heat to the BaAl₄ alloy alone but, more recently, it has become widespread to mix the BaAl₄ with an approximately equal weight of nickel. These two materials, in powder form, when heated react exothermically to form a solid residue of Ni-Al and evaporated Ba. However, these getter materials have to be heated to about 800°C before the exothermic reaction starts whereupon they reach 1000°C, and more, when there is the sudden release of heat on reacting exothermically.

In Japanese Patent Publication N° SHO 42-4123 the barium-aluminium (about 50% Ba) alloy is mixed with, preferably, 15% by weight of powdered tin to produce getters. Said getters are heated by means of high frequency electrical induction to about 600°C for one minute during the exhaust process. As a result of the reaction which may be produced by said heating, it is considered that BaSn₂ may be produced, or liberated barium is produced, from the barium-aluminium alloy by reaction of aluminium and tin. In either case, a mixed getter material of barium-aluminium alloy and tin which is stable at a normal temperature is activated and absorb gases at a normal temperature. Nevertheless there is a heating process involved which requires temperatures of several hundreds of degrees centigrade. Furthermore an uncontrolled chemical reaction is taking place.

Another family of getter devices has been based upon the elements zirconium or titanium. Powdered Zr 84% - Al 16%, Zr₂Fe nd Zr₂Ni are among these. They are known as non-evaporated getters because they do not require any of their component elements to be evaporated in order to become capable of sorbing gas. However they do require heating to a high temperature to make them gas sorptive. This is because they are covered with surface layers of oxides and nitrides which passivate them and render them inactive. Upon heating, in vacuum, the passivating layers diffuse into the bulk material and the surface becomes clean and active. This heating process usually takes place at a high temperature, say 900°C for about 10-30 seconds. This temperature can be reduced but requires a longer time. For instance several hours at 500°C.

Even more recently non-evaporated getters based on Zr-V have been used. Such alloys as Zr-V-Fe and Zr-V-Ni have gained widespread acceptance as "low temperature" activatable non-evaporated getters. By low temperature activatable it means that a significant proportion of their gettering activity already becomes available within a relatively short time at moderate temperatures. It is believed that this is due to the ease with which the surface layers of passivating materials may diffuse into the bulk material at these relatively low temperatures. Whatever the reason for their ability to become active at these relatively low temperatures of 400-500°C this can still be an undesirably high temperature under many circumstances. All these gas sorptive material have been used in admixture with other materials, both gas sorptive or not, in an attempt to lower their temperature of activation.

There are many occasions in which it is desirable to remove unwanted gases from a vessel which under no circumstances can be allowed to be subject to a high temperature. Such may be the case for instance when the vessel is made of organic plastic or contains components of organic plastic. The organic plastic may melt. Even if the organic plastics do not melt they may reach such a temperature that they start to decompose or at least give off a large amount of gas which may be hydrocarbons or other organic gases. If they are sorbed by the getter material, this causes their premature failure as they only have a finite gettering power or ability to sorb a fixed quantity of gas. The rapid sorption of a large amount of gas impairs their ability to later sorb gas during the life of the device in which they are employed. Otherwise there remains too high a gas pressure for the device to work as intended. This temperature may be as low as about 150°C. At these temperatures, and lower, oxygen and water vapour permeation, and especially nitrogen, can be a problem.

Lithium organic resins have been proposed for the sorption of gas impurities from impure gas streams, but they are used for the purification of nitrogen gas and not for its sorption, see US-A-4,603,148 and US-A-4,604,270.

Although it has been suggested that non-evaporated getters can be introduced into the device in a pre-activated form, that is when they have already been heated to a high temperature of about 600°C, they have already been subjected to many manufacturing processes such as grinding to fixed particle size, mixing with other materials, compaction or forming into pellets.

It is therefore an object of the present invention to provide a process for the sorption of residual gas in a vessel which is free from one or more of the disadvantages of prior art processes.

It is another object of the present invention to provide a process for the sorption of residual gas in a vessel which does not require the getter materials to be activated at temperatures greater than 150°C.

A further object of the present invention to provide a process for the sorption of unwanted gas in a vessel which does not require temperatures of greater than 150°C.

It is yet another object of the present invention to provide a process for the sorption of residual gas in a vessel which does not require the getter to be mixed with other materials.

Another object of the present invention to provide a process for the sorption of residual gas in a vessel which can be used in vessels made of organic plastic.

Yet a further object of the present invention is to provide a process for the sorption of nitrogen gas in a vessel made of organic plastic or which contains organic plastic.

These and other objects and advantages of the present invention will become clear to those skilled in the art by reference to the following description thereof and drawings wherein:
Fig. 1 is a drawing showing in a schematic form an apparatus for measuring the sorption properties of alloys useful in providing a process of the present invention,
Fig. 2 shows the results of sorption tests of N₂ at 25°C performed on alloy of BaLi₄ of the present invention,
Fig. 3 shows the results of sorption tests of various gases at 25°C performed on an alloy of BaLi₄ of the present invention;
Fig. 4 shows the results of sorption tests of N₂, at various temperatures, performed on an alloy of BaLi₄ of the present invention;
Fig. 5 shows the results of sorption tests of N₂ at 25°C performed on an alloy of BaLi₄ of the present invention;
Fig. 6 shows the gas sorption speed derived from the curves of Figs. 2-5 as a function of the quantity of gas sorbed;
Figs. 7-9 show the results of sorption tests of N₂ at 25°C performed on an alloy of Ba_{0.75}Ca_{0.25}Li₄ of the present invention;
Fig. 10 shows the gas sorption speed derived from the curves of Figs. 7-9 as a function of the quantity of nitrogen sorbed;
Figs. 11-15 show the results of sorption tests of N₂ at 25°C performed on an alloy of Ba_{0.5}Ca_{0.5}Li₄ of the present invention;
Fig. 16 shows the gas sorption speed derived from the curves of Figs. 11-15 as a function of the quantity of nitrogen sorbed;
Figs. 17-18 show the results of sorption tests of N₂ at 25°C performed on an alloy of BaLi₃Al of the present invention,
Fig. 19 shows the gas sorption speed derived from the curves of Figs. 17-18 as a function of the quantity of nitrogen sorbed; and
Fig. 20 shows the gas sorption speed of BaLi₄ and a traditional non-evaporated getter, for nitrogen, at various temperatures obtained by a different technique to that used for obtaining curves of Figs. 6, 10, 16 and 19.

The process of the present invention provides for the sorption of residual gas in a vessel by means of a non-evaporated barium getter. It comprises the steps of reducing an alloy of Ba₁₋ₓAₓLi_{4-y}B_{y}, preferably to a particle size of less than 5mm, under vacuum or an inert gas atmosphere and then placing the reduced alloy in the vessel. Upon exposing the reduced alloy to the residual gas in the vessel at a temperature of less than 150°C the gas is sorbed. The metal A is a metal chosen from the group consisting of elements of Group IIa of the periodic table of elements, excluding barium. The metal B is chosen from the group consisting of elements of Group IIIa of the periodic table of elements and magnesium.

The alloys of the present invention do not have to be activated, that is they are already capable of sorbing gases at room temperature and furthermore they do not have to be evaporated to produce a film of active material, such as barium before they sorb gas. Nevertheless they can be activated by heating to a temperature of not greater than 150°C. This could be between 50°C and 150°C for at least 10 minutes and then reducing the temperature to less than 50°C. The alloys can be described by the general formula Ba₁₋ₓAₓLi_{4-y}B_{y}, where A is a metal chosen from the group consisting of elements of Group IIa of the periodic table of elements, excluding barium. The numbering of the Groups of elements is that adopted by The American Chemical Society. Thus A can be calcium, magnesium and strontium but is preferably calcium as calcium is only slightly less reactive than barium. Magnesium and strontium are less preferred for their lower reactivity. The value of x may be as low as zero such that there is no metal of Group IIa present (except the barium). On the other hand it may be as high as 0.8. Above about 0.8 the alloy begins to lose its ability to react at room temperature with the residual gas at a sufficiently high sorption speed.

The element B is any metal chosen from the group consisting of elements Group IIIa of the periodic table of elements and magnesium. All members of Group IIIa can be adopted, for instance boron, but aluminium is preferred as it is readily available, it has a relatively high melting point and is extremely cheap, while gallium is liquid near ambient temperatures. Indium has a low melting point and is more expensive then aluminium. Tl is highly toxic. Furthermore 0≦y≦3.5.

These compounds can be easily comminuted or reduced to a particulate form without any difficulty. For instance they can be reduced to a particle size of less than 5 mm in diameter, and preferably less than 1 mm, by known techniques under a vacuum or inert atmosphere and then transferred to the vessel containing the unwanted gas which is desired to be removed. This is accomplished by placing the reduced alloy in the vessel and exposing the reduced alloy to the residual gas at room temperature.

The reduced alloy can be transferred to the vessel immediately but preferably takes place by means of an intermediate vessel in which the alloy is stored under vacuum or an inert atmosphere until it is required.

Surprisingly they immediately start to sorb large amounts of unwanted gas. Even more surprisingly they sorb nitrogen with a much higher sorption speed and sorb greater quantities than prior art non-evaporated getter devices after no activation, or an activation at not greater than 150°C.

The invention may be better understood by reference to the following examples wherein all parts and percentages are by weight unless otherwise indicated. These examples are designed to teach those skilled in the art how to practice the present invention and represent the best mode presently known for practicing the invention.

### EXAMPLE 1

This example is not representative of the present invention but is designed to show an apparatus suitable for measuring the gas sorption properties of alloys suitable for practicing processes of the present invention. Fig. 1 is a drawing showing in a schematic form an apparatus 100 for measuring the sorptive properties of Ba₁₋ₓAₓLi_{4-y}B_{y} alloys useful in the present invention. A vacuum pumping system 102 is connected by means of a first valve 104 to a dosing volume 106. Connected with dosing volume 106 there is a series of second valves 110, 110', 110'' for the inlet of test gases from a series of test gas reservoirs 112, 112', 112'', containing N₂, artificial air, and CO respectively, and a pressure measuring gauge 114. To dosing volume 106 is also connected, by third valve 116, a test chamber 118 containing the sample 120 under test.

In operation valves 110, 110', 110'' and 116 are closed and 104 is opened and the vacuum pump system 102 pumped the system down to 10⁻⁶ mbar. For all test the dosing volume 106 was a volume of 0.71 litre. A sample of powered alloy 120, contained within a glass bulb test chamber 118 of approximately 0.1-0.3 litre volume (depending upon the sample), under an inert atmosphere of argon gas was attached to apparatus 100 via valve 116 (closed). Valve 116 was opened and again the system was pumped down to 10⁻⁶ mbar while the sample was held at about 100°C for 20 minutes which simulates a process to which the getter may be subject. Valves 104 and 116 were then closed and test gas was admitted to dosing volume 106, from gas reservoir 112, (112', 112'') by opening valve 110 (110', 110'') for a short while. The pressure was noted on pressure gauge 114, and was arranged to be such that the pressure was about 0.4-1.0 mbar after opening valve 116 to introduce a dose of test gas to the sample 120.

### EXAMPLE 2

This example was designed to show how to manufacture an alloy useful in the process of the present invention.

In an iron crucible were placed 155.88g of commercial grade barium (purity greater than 98%) obtained from Degussa together with 11.3 g of lithium. The crucible was placed in an induction furnace and heated under an argon atmosphere at 400 mbar pressure with medium frequency induction heating until the mixture was thoroughly melted and homogeneous thus forming a fusion. The fusion was then poured into a cold copper mould and allowed to cool to room temperature while still under the protective atmosphere of argon.

The alloy corresponds to the intermetallic compound BaLi₄.

### EXAMPLE 3

This example was designed to show the use of an alloy in the process of the present invention.

A barium-lithium alloy as prepare in Example 2 above was placed in a glove-box under a protective atmosphere of argon at slightly greater than 1 atmosphere pressure. The alloy was ground using a mortar and pestle to a particle size of less than 1mm and a sample of 2.7 g was sealed in a glass vessel of volume 0.17 litre. The sample in the glass vessel was then attached as test chamber 118 to the test apparatus of Example 1. The procedure of Example 1 was followed and a first dose of gas, in this case nitrogen (from reservoir 112 by means of valve 110), was introduced to the sample. The pressure in the vessel was measured by means of pressure gauge 114 as a function of time. The curve obtained is reported on Fig. 2 as curve 1. The sorption was so rapid that the pressure drop was almost instantaneous. A second dose of nitrogen was introduced and the pressure in the vessel as measured by the pressure gauge 114 was reported as curve 2 on Fig. 2.

The gas was replaced by artificial air, that is a mixture of 80% v/v N₂ + 20% v/v O₂ (from reservoir 112' by means of valve 110') and the pressure in the vessel was recorded as curve 3 on Fig. 3. This was repeated to give curve 4. The gas was replaced by CO (from reservoir 112'' by means of valve 110'') and the pressure in the vessel was recorded as curve 5 for which the sorption was so rapid that the pressure drop was almost instantaneous. Artificial air was again introduced to give curve 6.

The sample was then cooled to 0°C and on introducing a sample of N₂ gas curve 7 was recorded.

The sample was then cooled to about -8°C to -9°C with a bath of alcohol + iced water and on introducing a dose of nitrogen curve 8 was recorded.

Again at 25°C a dose of nitrogen was introduced and curve 9 was recorded.

A further 3 doses of nitrogen were introduced to the sample and curves 10-12 were recorded.

The total doses of gas absorbed by the sample during these tests were, N₂ = 2818 mbar.cm³; O₂ = 421 mbar.cm³; CO = 216 mbar.cm³.

Fig. 6 shows the gas sorption speed derived from the curves of Figs. 2-5, by differentiation, as a function of gas sorbed.

### EXAMPLE 4

This example was designed to show how to manufacture another alloy, by partial replacement of barium by calcium, useful in the process of the present invention.

114.08 g of barium (type HP made by SAES Getters S.p.A.) was placed in an iron crucible together with 30.75 g of lithium and 1.10 g of granulated calcium (supplied by Carlo Erba, purity greater than 99.5%).

The crucible was placed in an induction furnace and heated under an argon atmosphere of 400 mbar with medium frequency induction heating until the mixture was thoroughly melted and homogeneous thus forming a fusion. The fusion was then poured into a cold iron mould and allowed to cool to room temperature while still under the protective atmosphere of argon. The weight of alloy after fusion was 138 g.

The alloy corresponds to the composition Ba_{0.75}Ca_{0.25}Li₄.

### EXAMPLE 5

This example was designed to show the use of the alloy produced as in Example 4 in the process of the present invention.

A barium-calcium-lithium alloy as prepared in Example 4 above was placed in a glove box under a protective atmosphere of argon at slightly greater than 1 atmosphere pressure. The alloy was ground to a particle size of less than 1 mm with a pestle and a mortar and a sample of 2.0 g was sealed in a glass vessel of volume 0.32 litre. The sorption properties were measured as in Example 3 for N₂ at 25°C and are reported as curves 1-14 in Figs. 7-9. Fig. 10 shows the nitrogen sorption speed derived from the curves of Figs. 7-9, by differentiation, as a function of nitrogen sorbed.

### EXAMPLE 6

This example was designed to show how to manufacture another alloy, by replacement of more barium by calcium, useful in the process of the present invention.

25.3 g of barium (type HP made by SAES Getters S.p.A.) was placed in an iron crucible together with 7.38 g of granulated calcium (purity greater than 99.5%) obtained from Carlo Erba and 10.23 g of lithium. The crucible was placed in an induction furnace and heated under an argon atmosphere at 400 mbar pressure with medium frequency induction heating until the mixture was thoroughly melted and homogeneous thus forming a fusion. The fusion was then poured into a cold iron mold and allowed to cool to room temperature while still under the protective atmosphere of argon. The weight of alloy after fusion was 39.6 g.

The alloy corresponds to a composition Ba_{0.5}Ca_{0.5}Li₄.

### EXAMPLE 7

This example was designed to show- the use of the alloy produced as in Example 6 in the process of the present invention.

A barium-calcium lithium alloy as prepared in Example 6 above was placed in a glove box under a protective atmosphere of argon at slightly greater than 1 atmosphere pressure. The alloy was ground to a particle size of less than 1 mm with a pestle and mortar and a sample of 2.47 g was sealed in a glass vessel of volume 0.15 litre. The sorption properties were measured for nitrogen at 25°C as in Example 3, and are reported as curves 1-28 in Figs. 11-15. Fig. 16 shows the gas sorption speed derived from the curves of Figs. 11-15 as a function of quantity of gas sorbed.

### EXAMPLE 8

This example was designed to show how to manufacture yet another alloy useful in the process of the present invention.
59.14 g of barium (type HP made by SAES Getters S.p.A.) was placed in an iron crucible together with 8.97 g of lithium and 11.61 g of SAVA aluminium beads (purity greater than 98.5%).

The crucible was placed in an induction furnace and heated under an argon atmosphere of 400 mbar with medium frequency induction heating until the mixture was thoroughly melted and homogeneous thus producing a fusion. The fusion was then poured into a cold iron mold and allowed to cool to room temperature while still under the protective atmosphere of argon. The weight of alloy after fusion was 78.3 g.

The alloy corresponds to the composition BaLi₃Al.

### EXAMPLE 9

This example was designed to show the use of the alloy produced as in Example 8 in the process of the present invention.

A barium-lithium-aluminium alloy as prepared in Example 8 above was placed in a glove box under a protective atmosphere of argon at slightly greater than 1 atmosphere pressure. The alloy was ground to a particle size of less than 1 mm with a pestle and a mortar and a sample of 2.4 g was sealed in a glass vessel of volume 0.32 litre. The sorption properties were measured as in Example 3 for N₂ at 25°C and are reported as curves 1-7 in Figs. 17-18. Fig. 19 shows the gas sorption speed derived from the curves of Figs. 17-18, by differentiation, as a function of gas sorbed.

### EXAMPLE 10

This example was designed to show the N₂ sorption properties of a prior art alloy. A low temperature activatable non-evaporated of 70% Zr - 24.6% V - 5.4% Fe (nominal weight composition) of weight 100 mg was activated by heating to 450°C for 10 minutes under vacuum at better than 10⁻³ mbar and then caused to sorb N₂ at 25°C at a pressure of about 10⁻⁵ mbar in an apparatus described in the ASTM F798-82 Standard Practice for Determining Gettering Rate, Sorption Capacity, and Gas Content of Nonevaporable Getters in the Molecular Flow Region. The gettering rate (sometimes called sorption speed) was plotted against the quantity sorbed, for the equivalent 2g getter, to give curve A on Fig. 20.

The test was repeated using a sorption temperature of 350°C and the curve of nitrogen sorption, again for the equivalent 2g getter was plotted as curve B of Fig. 20.

### EXAMPLE 11

This example was designed to show the N₂ sorption properties of an alloy according to the present invention. A barium-lithium alloy as prepared in Example 2 above was prepared and 2g, having a particle size of less than 1mm, was placed in the same ASTM apparatus used for Example 10. After being held at a temperature of 100°C for 15-20 minutes, which simulates a process to which the getter may be subjected the getter was cooled to 25°C and its curve of nitrogen sorption was plotted as curve C on Fig. 20. After the getter had sorbed a quantity of gas the flow was interrupted. On continuing, the curve C' was obtained, and successively with curves C'' and C'''.

### EXAMPLE 12

The Example 11 was repeated except that the getter was activated at a temperature of 130°C for 3 hours followed by 100°C for 16 hours and the getter was held at 80°C while sorbing nitrogen.

The gettering rate was again plotted against quantity sorbed to give curve D on Fig. 20.

### DISCUSSION

By comparison of curve C with curve A of Fig. 20, and D with B, it is seen that alloys used in processes of the present invention have a higher gettering rate (sorption speed) when they have sorbed a greater quantity of nitrogen than traditional getter alloys. Furthermore these properties are obtained after activation at much lower temperatures.

In addition Figs. 6, 10, 16 and 19 show a remarkable ability for the large quantities of N₂ and other gases sorbed.

Although the invention has been described in considerable detail with reference to certain preferred embodiments designed to teach those skilled in the art how best to practice the invention, it will be realized that other modifications may be employed without departing from the scope of the appended claims.

For instance, it will be realized that small amounts of lithium can be replaced by other elements of the alkali metal series of elements, and notably sodium and potassium without substantially affecting their properties. Furthermore although the invention has been described and exemplified in terms of the stoichiometric compound BaLi₄ some degree of departure from stoichiometry will be allowed within the formula Ba₁₋ₓAₓLi_{4-y}B_{y}.

## Claims

1. A process for the sorption of residual gas in a vessel by a non-evaporated barium getter comprising the steps of:
i) reducing an alloy of Ba₁₋ₓAₓLi_{4-y}B_{y} to particles under a vacuum or inert gas to produce a reduced alloy;
ii) placing the reduced alloy in the vessel; and
iii) exposing the reduced alloy to the residual gas at a temperature of less than 150°C,
wherein,
A is a metal chosen from the group consisting of elements of Group IIa of the periodic table of elements, excluding barium,
B is a metal chosen from the group consisting of elements of Group IIIa, of the periodic table of elements and magnesium,$\begin{matrix}\begin{matrix}\text{0 ≦ x ≦ 0.8, and} \\ \text{0 ≦ y ≦ 3.5,}\end{matrix}\end{matrix}$ wherein the numbering of the Groups of the elements is that adopted by the American Chemical Society.

2. A process of Claim 1 in which step iii) includes exposing the reduced alloy to the residual gas at a temperature of between 50° and 150°C for at least 10 minutes and then reducing the temperature to less than 50°C.

3. A process of Claim 1 in which A is a metal chosen from the group consisting of magnesium, calcium and strontium.

4. A process of Claim 1 in which B is a metal chosen from the group consisting of boron, aluminium and magnesium.

5. A process of Claim 1 in which 0≦x≦0.5

6. A process of Claim 1 in which the non-evaporated barium getter comprises the alloy BaLi₄.

7. A process of Claim 1 in which the non-evaporated barium getter comprises the alloy Ba_{0.75}Ca_{0.25}Li₄.

8. A process of Claim 1 in which the non-evaporated barium getter comprises the alloy Ba_{0.5}Ca_{0.5}Li₄.

9. A process of Claim 1 in which the non-evaporated barium getter comprises the alloy BaLi₃Al.

10. A process of Claim 1 in which the reduced alloy has a particle size of less than 5mm.

11. A process of Claim 10 in which the reduced alloy has particle size of less than 1mm.

12. A process for the sorption of residual gases in a vessel by a non-evaporated barium getter comprising the steps of:
i) comminuting an alloy of Ba₁₋ₓAₓLi_{4-y}B_{y} to particle in the absence of reactive gases to produce a particulate alloy;
ii) placing the particulate alloy in the vessel; and
iii) exposing the particulate alloy to the residual gas at a temperature of less than 150°C; wherein:
"A" is a metal selected from the group consisting of magnesium calcium, and strontium;
"B" is a metal selected from the group consisting of boron, aluminum, and magnesium;
"x" has a value from zero to 0.8; and
"y" has a value from zero to 3.5.

13. A process for the sorption of residual gases in a vessel by a non-evaporated barium getter comprising the steps of:
i) comminuting an alloy of BaLi₄ to particles in the absence of reactive gases to produce a particulate alloy;
ii) placing the particulate alloy in the vessel; and
iii) exposing the particulate alloy to the residual gas at a temperature of less than 150°C.

14. A process for the sorption of residual gases at temperatures less than 150°C in a closed vessel, the interior walls of which are free of a barium film, by contacting the residual gases with a particulate alloy of Ba₁₋ₓAₓLi_{4-y}B_{y}, wherein:
the particulate alloy has a particle size less than 5mm;
sorption of residual gases occurs at the surface of the particles;
"A" is a metal selected from the group consisting of magnesium, calcium and strontium;
"B" is a metal selected from the group consisting of boron, aluminum and magnesium;
"x" has a value from zero to 0.8; and
"y" has a value from zero to 3.5.

## Patentansprüche

1. Verfahren zur Sorption von Rückstandsgas in einem Behälter durch nicht-verdampftes Bariumgetter, umfassend die Schritte:
i) Reduzieren einer Legierung Ba₁₋ₓAₓLi_{4-y}B_{y} zu Teilchen unter einem Vakuum- oder Inertgas zur Erzeugung einer reduzierten Legierung;
ii) Einsetzen der reduzierten Legierung in einen Behälter;
iii) Aussetzen der reduzierten Legierung einem Rückstandsgas bei einer Temperatur von weniger als 150 °C,
wobei
A ein Metall ist, ausgewählt aus der Gruppe bestehend aus den Elementen der Gruppe IIa des periodischen Systems der Elemente, ausgenommen Barium,
B ein Metall ist, ausgewählt aus der Gruppe, bestehend aus den Elementen der Gruppe IIIa des periodischen Systems der Elemente und Magnesium,
mit$\begin{matrix}\begin{matrix}\text{0 ≦ x ≦ 0,8 und} \\ \text{0 ≦ y ≦ 3,5}\end{matrix}\end{matrix}$ wobei die Numerierung der Gruppen der Elemente die von der American Chemical Society eingeführte ist.

2. Verfahren nach Anspruch 1, bei dem der Schritt iii) das Aussetzen der reduzierten Legierung einem Rückstandsgas bei einer Temperatur zwischen 50 und 150 °C für wenigstens 10 Minuten einschließt und dann Absenken der Temperatur auf unter 50 °C.

3. Verfahren nach Anspruch 1, bei dem A ein Metall ist, ausgewählt aus der Gruppe bestehend aus Magnesium, Calcium und Strontium.

4. Verfahren nach Anspruch 1, bei dem B ein Metall aus der Gruppe bestehend aus Bor, Aluminium und Magnesium ist.

5. Verfahren nach Anspruch 1, bei dem 0 ≦ x ≦ 0,5 ist.

6. Verfahren nach Anspruch 1, bei dem das nicht verdampfte Bariumgetter die Legierung BaLi₄ umfasst.

7. Verfahren nach Anspruch 1, bei dem das nicht verdampfte Bariumgetter die Legierung Ba_{0,75}Ca_{0,25}Li₄ umfasst.

8. Verfahren nach Anspruch 1, bei dem das nicht verdampfte Bariumgetter die Legierung Ba_{0,5}Ca_{0,5}Li₄ umfasst.

9. Verfahren nach Anspruch 1, bei dem das nicht verdampfte Bariumgetter die Legierung BaLi₃Al umfasst.

10. Verfahren nach Anspruch 1, bei dem die reduzierte Legierung eine Teilchengröße von weniger als 5 mm hat.

11. Verfahren nach Anspruch 10, bei dem die reduzierte Legierung eine Teilchengröße von weniger als 1 mm hat.

12. Verfahren zur Sorption von Rückstandsgas in einem Behälter durch ein nicht verdampftes Bariumgetter, umfassend die Schritte:
i) Zerkleinern einer Legierung Ba₁₋ₓAₓLi_{4-y}B_{y} zu Teilchen in Abwesenheit von reaktiven Gasen zur Erzeugung einer gekörnten Legierung;
ii) Einsetzen der gekörnten Legierung in einen Behälter; und
iii) Aussetzen der zerkleinerten Legierung zu einem Rückstandsgas bei einer Temperatur von weniger als 150 °C; wobei:
"A" ein Metall ist, ausgewählt aus der Gruppe bestehend aus Magnesium, Calcium und Strontium;
"B" ein Metall ist, ausgewählt aus der Gruppe bestehend aus Bor, Aluminium und Magnesium;
"x" einen Wert von 0 bis 0,8 hat; und
"y" einen Wert von 0 bis 3,5 hat.

13. Verfahren zur Sorption von Rückstandsgasen in einem Behälter durch nicht verdampftes Bariumgetter, umfassend die Schritte:
i) Zerkleinern einer Legierung von BaLi₄ zu Teilchen in Abwesenheit von reaktiven Gasen zur Erzeugung einer gekörnten Legierung;
ii) Einsetzen der gekörnten Legierung in einen Behälter; und
iii) Aussetzen der gekörnten Legierung Zu einem Rückstandsgas bei einer Temperatur von unter 150 °C.

14. Verfahren zur Sorption von Rückstandsgasen bei Temperaturen von weniger als 150 °C in einem geschlossenen Behälter, dessen innere Wände frei einem Bariumfilm sind, durch Kontaktieren der Rückstandsgase mit der gekörnten Legierung Ba₁₋ₓAₓLi_{4-y}B_{y}, wobei die gekörnte Legierung eine Teilchengröße von weniger als 5 mm hat; Sorption der Rückstandsgase tritt auf an der Oberfläche der Teilchen; und
"A" ein Metall ist, ausgewählt aus der Gruppe, bestehend aus Magnesium, Calcium und Strontium;
"B" ein Metall ist, ausgewählt aus der Gruppe, bestehend aus Bor, Aluminium und Magnesium;
"x" einen Wert von 0 bis 0,8 hat; und
"y" einen Wert von 0 bis 3,5 hat.

## Revendications

1. Un procédé pour l'absorption de gaz résiduels d'un récipient par un getter non évaporé au baryum comprenant les opérations consistant à :
i) réduire un alliage de Ba₁₋ₓAₓLi_{4-y}B_{y} en particules sous vide ou en présence d'un gaz inerte pour produire un alliage réduit ;
ii) placer l'alliage réduit dans le récipient ; et
iii) exposer l'alliage réduit aux gaz résiduels à une température inférieure à 150 °C,
dans lequel
A. est un métal choisi dans le groupe comprenant des éléments du Groupe IIa du tableau périodique des éléments, en excluant le baryum,
B. est un métal choisi dans le groupe comprenant des éléments du Groupe IIIa du tableau périodique des éléments et le magnésium,
$\begin{matrix}\begin{matrix}\text{0 ≦ x ≦ 0,8, et} \\ \text{0 ≦ y ≦ 3,5,}\end{matrix}\end{matrix}$ où la numérotation des Groupes des éléments est celle adoptée par l'American Chemical Society.

2. Un procédé de la revendication 1, dans lequel l'opération iii) comprend le fait d'exposer l'alliage réduit aux gaz résiduels à une température entre 50° et 150°C pendant au moins 10 minutes et réduire alors la température à moins de 50°C.

3. Un procédé de la revendication 1, dans lequel A est un métal choisi dans le groupe comprenant le magnésium, le calcium et le strontium.

4. Un procédé de la revendication 1, dans lequel B est un métal choisi dans le groupe comprenant le bore, l'aluminium et le magnésium.

5. Un procédé de la revendication 1, dans lequel 0 ≦ x ≦ 0,5.

6. Un procédé de la revendication 1, dans lequel le getter non évaporé au baryum comprend l'alliage BaLi₄.

7. Un procédé de la revendication 1, dans lequel le getter non évaporé au baryum comprend l'alliage Ba_{0,75}Ca_{0,25}Li₄.

8. Un procédé de la revendication 1, dans lequel le getter non évaporé au baryum comprend l'alliage Ba_{0,5}Ca_{0,5}Li₄.

9. Un procédé de la revendication 1, dans lequel le getter non évaporé au baryum comprend l'alliage BaLi₃Al.

10. Un procédé de la revendication 1, dans lequel l'alliage réduit présente une granulométrie inférieure à 5 mm.

11. Un procédé de la revendication 10, dans lequel l'alliage réduit présente une granulométrie inférieure à 1 mm.

12. Un procédé pour l'absorption de gaz résiduels dans un récipient par un getter non évaporé au baryum comprenant les opérations consistant à :
i) broyer un alliage de Ba₁₋ₓAₓLi_{4-y}B_{y} en fines particules en l'absence de gaz réactifs afin de produire un alliage particulaire ;
ii) placer l'alliage particulaire dans le récipient ; et
iii) exposer l'alliage particulaire aux gaz résiduels à une température inférieure à 150 °C ; dans lequel :
"A" est un métal choisi dans le groupe comprenant le magnésium, le calcium et le strontium ;
"B" est un métal choisi dans le groupe comprenant le bore, l'aluminium et le magnésium ;
"x" présente une valeur de zéro à 0,8 ; et
"y" présente une valeur de zéro à 3,5.

13. Un procédé pour l'absorption de gaz résiduels dans un récipient par un getter non évaporé au baryum comprenant les opérations consistant à :
i) broyer un alliage de BaLi₄ en fines particules en l'absence de gaz réactifs pour produire un alliage particulaire ;
ii) placer l'alliage particulaire dans le récipient ; et
iii) exposer l'alliage particulaire aux gaz résiduels à une température inférieure à 150°C.

14. Un procédé pour l'absorption de gaz résiduels à des températures inférieures à 150°C dans un récipient fermé, dont les parois intérieures sont exemptes d'une couche mince de baryum, en mettant en contact les gaz résiduels avec un alliage particulaire de Ba₁₋ₓAₓLi_{4-y}B_{y}, dans lequel :
l'alliage particulaire présente une granulométrie inférieure à 5 mm ;
l'absorption des gaz résiduels se produit à la surface des particules ;
"A" est un métal choisi dans le groupe comprenant le magnésium, le calcium et le strontium ;
"B" est un métal choisi dans le groupe comprenant le bore, l'aluminium et le magnésium ;
"x" présente une valeur de zéro à 1,8 ; et
"y" présente une valeur de zéro à 3,5.
